

## UNITED STATES PATENT OFFICE.

THOMAS PHILIP THOMAS, OF BLOOMFIELD, NEW JERSEY, ASSIGNOR TO WESTINGHOUSE LAMP COMPANY, A CORPORATION OF PENNSYLVANIA.

## ELECTRON-EMISSION MATERIAL AND THE ACTIVATION THEREOF.

No Drawing.

Application filed April 14, 1923. Serial No. 632,168.

This invention relates to material for electron-emission purposes and more particularly to the application of a thorium compound to filamentary material and the decomposition thereof by heat to develop thorium thereon.

An object of my invention is the formation of a coating of metallic thorium on material for electron-emission purposes, by the direct application thereto of a thorium compound and the decomposition thereof by heat to yield free thorium.

Another object of my invention is the activation of material serving as the hot cathode of an electron device by the direct application thereto of thorium oxalate or the like and heating, whereby free thorium is developed thereon, or the application of such to an adjacent electrode or plate, whereby the cathode is activated by heating the plate to decompose the oxalate or the like and transfer liberated thorium to the cathode.

A further object of my invention is the preparation of activated electron-emission material by the application thereto of thorium oxalate held thereon by a suitable binder, such as an amyl-acetate solution of nitro-cellulose, and heating the same to cause a decomposition thereof in place, to leave free thorium on the surface of the material.

A still further object of my invention is the manufacture of electron devices comprising an electron-emitting filament consisting of a refractory metal filament coated with thorium oxalate, held thereon by a suitable binder, and adapted to be decomposed to yield free thorium for activation and gaseous carbon compounds which are eliminated by a suitable metallic clean-up agent.

Other objects and advantages of my invention will become apparent from the following description.

Metallic thorium, as is well known, has a high electron emissivity and, for this reason, various methods have been devised for coating material, designed for electron-emission purposes, with metallic thorium, to "activate" or increase the electron-emissivity thereof. For example, in the copending application of Ralph E. Myers, Serial No. 578,470, filed July 29, 1922, activation of thoriated filaments and assigned to the

Westinghouse Lamp Company, is disclosed a method whereby thorium is finally developed on thoriated wire composed of 55 tungsten or the like, by heating the same in a hydro-carbon atmosphere, although some intermediate product or products may be formed by this process.

When a filament so treated is finally 60 heated, as the hot cathode in an electron-device, metallic thorium is developed in or on the filament, either having been formed by the reducing action of the hydro-carbon or by carbon absorbed therefrom when the 65 wire is first heated within the hydro-carbon atmosphere. Such method has given very good results in practice, but it entails a preliminary heating operation of the filamentary material, prior to its introduction into 70 an electron device. That is, the filamentary material is heated in a hydro-carbon atmosphere to precondition it for the development of thorium thereon when used as the hot cathode in an electron device.

According to my invention, I obviate the necessity of the preliminary heat treatment by applying, to the filamentary material, a compound of thorium, decomposable by heat to yield free thorium on the surface of the 80 filamentary material. The preferred material used for this purpose is thorium oxalate, although I do not wish to be restricted to the precise compound mentioned, as any solid thorium compound, which decomposes on 85 heating to liberate free thorium therefrom before it evaporate, may be employed for this purpose. The thorium oxalate, in powdered form, is preferably mixed with a suitable binder solution, for example, nitro-cellulose dissolved in amyl-acetate, and applied to the filamentary material as a paint or varnish, but any other method suitable for affixing the thorium compound firmly to the filamentary material may be employed.

The material so treated may then be attached to a suitable mount including a plate, to which is preferably attached metallic clean-up material, such as aluminum, magnesium or both and introduced into an evacuated envelope as the hot cathode or electron-emitting filament of an electron device. The plate may then be heated in any desired manner, after the device is evacuated, for



clean-up material therein to eliminate residual gases and such carbon compounds.

3. The method of activating filamentary material for electron-emission purposes comprising enclosing the same in an evacuated envelope as a cathode with an anode one of which is coated with thorium oxalate and heating the coated member to decompose

the oxalate, liberate free thorium and causing the filamentary material to be coated therewith.

In testimony whereof, I have hereunto subscribed my name this 13th day of April, 1923.

THOMAS PHILIP THOMAS.